



US006248028B1

(12) **United States Patent**  
Higuchi et al.

(10) **Patent No.:** US 6,248,028 B1  
(45) **Date of Patent:** \*Jun. 19, 2001

(54) **MULTI-PIECE SOLID GOLF BALL**

(75) Inventors: **Hiroshi Higuchi; Yasushi Ichikawa; Hisashi Yamagishi; Junji Hayashi; Akira Kawata**, all of Chichibu (JP)

(73) Assignee: **Bridgestone Sports Co., Ltd.**, Tokyo (JP)

(\*) Notice: Subject to any disclaimer, the term of this patent is extended or adjusted under 35 U.S.C. 154(b) by 0 days.

This patent is subject to a terminal disclaimer.

(21) Appl. No.: **09/130,877**

(22) Filed: **Aug. 7, 1998**

**Related U.S. Application Data**

(60) Provisional application No. 60/058,566, filed on Sep. 11, 1997.

**Foreign Application Priority Data**

Aug. 8, 1997 (JP) ..... 9-227607  
Oct. 22, 1997 (JP) ..... 9-307969

(51) **Int. Cl.**<sup>7</sup> ..... **A63B 37/06**  
(52) **U.S. Cl.** ..... **473/374; 473/373**  
(58) **Field of Search** ..... 473/351, 373, 473/374, 377, 378

**References Cited**

## U.S. PATENT DOCUMENTS

4,674,751 6/1987 Molitor et al. .



4,919,434 \* 4/1990 Saito ..... 473/373  
5,026,067 6/1991 Gentilumo .  
5,553,852 \* 9/1996 Higuchi et al. ..... 473/373  
5,730,664 \* 3/1998 Asakura et al. ..... 473/373  
5,813,923 \* 9/1998 Cavallaro et al. ..... 473/374  
5,929,189 \* 7/1999 Ichikawa et al. ..... 473/374 X

## FOREIGN PATENT DOCUMENTS

0 633 043 A1 1/1995 (EP) .  
0 637 459 A1 2/1995 (EP) .  
WO 97/18861 5/1997 (WO) .

\* cited by examiner

*Primary Examiner*—Mark S. Graham

*Assistant Examiner*—Raeann Gorden

(74) *Attorney, Agent, or Firm*—Sughrue, Mion, Zinn, Macpeak & Seas, PLLC

(57)

**ABSTRACT**

A multi-piece solid golf ball featuring an increased flight distance, superior control, good feeling, and improved durability is provided. A multi-piece solid golf ball comprising a solid core and a cover of two inner and outer layers surrounding the core is characterized in that the solid core has a distortion of at least 2.7 mm under an applied load of 100 kg, the inner cover layer is formed mainly of a thermoplastic polyester elastomer to a Shore D hardness of 28-58, and the outer cover layer is formed mainly of a thermoplastic polyurethane elastomer to a Shore D hardness of 30-55.

**14 Claims, 1 Drawing Sheet**

FIG. 1



**MULTI-PIECE SOLID GOLF BALL****CROSS REFERENCE TO RELATED APPLICATION**

This application is an application filed under 35 U.S.C. §111(a) claiming benefit pursuant to 35 U.S.C. § 119(e)(i) of the filing date of the Provincial Application 60/058,566 filed on Sep. 11, 1997 pursuant to 35 U.S.C. §111 (b).

**BACKGROUND OF THE INVENTION****1. Field of the Invention**

This invention relates to a multi-piece solid golf ball comprising a solid core enclosed with a cover of two inner and outer layers.

**2. Prior Art**

Golf balls of various structures have recently been proposed. In particular, many proposals were made on solid golf balls, *inter alia*, multi-piece solid golf balls comprising a solid core enclosed with a cover of plural layers from the standpoints of flight distance, control (or spin rate), and feeling (see JP-A 244174/1992, 142228/1994, 24084/1995, 24085/1995, and 10358/1997).

Nevertheless, there is a desire to have a multi-piece solid golf ball having further improved flight performance, superior spin property, and good feeling upon wood, iron and putter shots as well as good scraping resistance and durability.

**SUMMARY OF THE INVENTION**

Making extensive investigations to meet the above desire, the inventors have found that it is effective for a multi-piece solid golf ball comprising a solid core and a cover of two layers, an inner and outer layers surrounding the core that the solid core is formed relatively soft, the inner cover layer is formed mainly of a thermoplastic polyester elastomer, the outer cover layer is formed mainly of a thermoplastic polyurethane elastomer, the inner cover layer has a Shore D hardness of 28 to 58, and the outer cover layer has a Shore D hardness of 30 to 55.

Specifically, the present invention provides:

- (1) A multi-piece solid golf ball comprising a solid core and a cover of two inner and outer layers surrounding the core, characterized in that said solid core has a distortion of at least 2.7 mm under an applied load of 100 kg, said inner cover layer is formed mainly of a thermoplastic polyester elastomer to a Shore D hardness of 28 to 58, and said outer cover layer is formed mainly of a thermoplastic polyurethane elastomer to a Shore D hardness of 30 to 55.
- (2) The golf ball of (1) wherein the ball as a whole has an inertia moment of at least 83 g-cm<sup>2</sup>.
- (3) The golf ball of (1) or (2) wherein up to 30% by weight of an inorganic filler is added to said outer cover layer.
- (4) The golf ball of any one of (1) to (3) wherein said inner cover layer contains 0 to 30% by weight of an inorganic filler.
- (5) The golf ball of any one of (1) to (4) wherein said outer cover layer has a specific gravity of 1.05 to 1.4.
- (6) The golf ball of any one of (1) to (5) wherein said inner cover layer has a specific gravity of 1.05 to 1.4.
- (7) The golf ball of any one of (1) to (6) wherein said core has a specific gravity of 0.9 to 1.2.

(8) The golf ball of any one of (1) to (7) wherein said outer cover layer has a gage of 0.5 to 2.5 mm, said inner cover layer has a gage of 0.5 to 3.0 mm, and said cover has a total gage of 1.0 to 5.5 mm.

5 The golf ball of the invention features an increased flight distance, superior control upon iron shots, good feeling upon shots with any club of wood, iron and putter, high resistance to scraping upon control shots with an iron, and good durability.

**BRIEF DESCRIPTION OF THE DRAWING**

FIG. 1 is a schematic cross-section of a three-piece gold ball according to the invention.

**DETAILED DESCRIPTION OF THE INVENTION**

Now the invention is described in more detail.

10 The multi-piece solid golf ball of the invention has a solid core 1 and a cover 4 surrounding the core of a two-layer structure of inner and outer cover layers 2 and 3.

15 The solid core used herein is formed mainly of a rubber base. Natural rubber and/or synthetic rubber which is used in conventional solid golf balls can be used as the rubber base although 1,4-polybutadiene having at least 40% of a cis structure is especially preferred in the practice of the invention. Herein, natural rubber, polyisoprene rubber, styrene-butadiene rubber or the like may be blended with the polybutadiene rubber if desired.

20 More particularly, the solid core 1 of the golf ball according to the invention is obtained in conventional ways by adjusting vulcanizing conditions and blending ratio. In general, the solid core composition contains a base rubber, a crosslinking agent, a co-crosslinking agent, an inert filler, etc.

25 The base rubber used may be the above-mentioned natural rubber and/or synthetic rubber. The crosslinking agent is exemplified by organic peroxides such as dicumyl peroxide and di-t-butyl peroxide, with the dicumyl peroxide being especially preferred. The amount of the crosslinking agent blended is usually 0.5 to 2.0 parts by weight per 100 parts by weight of the base rubber.

30 The co-crosslinking agent is not critical and exemplified by metal salts of unsaturated fatty acids, especially zinc and magnesium salts of unsaturated fatty acids having 3 to 8 carbon atoms (e.g., acrylic acid and methacrylic acid), with zinc acrylate being especially preferred. The amount of the co-crosslinking agent blended is 10 to 50 parts by weight, preferably 20 to 48 parts by weight per 100 parts by weight of the base rubber.

35 Examples of the inert filler include zinc oxide, barium sulfate, silica, calcium carbonate, and zinc carbonate, with zinc oxide and barium sulfate being commonly used. The amount of the filler blended is governed by the specific gravity of the core and the cover, the weight specification of the ball, etc. and not critical although it is usually 1 to 30 parts by weight per 100 parts by weight of the base rubber. It is understood that in the practice of the invention, the solid core is given an optimum hardness by properly adjusting the amount of zinc oxide and barium sulfate blended.

40 A solid core composition is prepared by kneading the above-mentioned components in a conventional mixer such as a Banbury mixer and roll mill, and it is compression or injection molded in a core mold. The molding is then cured into a solid core by heating at a sufficient temperature for the crosslinking agent and co-crosslinking agent to function (for example, about 130 to 170° C. when dicumyl peroxide and

zinc acrylate are used as the crosslinking agent and the co-crosslinking agent, respectively.

The solid core **1** should have a distortion or deformation of at least 2.7 mm, preferably 2.8 to 6.0 mm, more preferably 2.9 to 5.0 mm under an applied load of 100 kg. A distortion of less than 2.7 mm under an applied load of 100 kg (hard core) would give disadvantages such as a hard hitting feel. A too much distortion (too soft core) would sometimes result in poor restitution.

The solid core preferably has a specific gravity of 0.9 to 1.2, especially 1.01 to 1.18.

In the practice of the invention, the solid core **1** preferably has a diameter (**2**) of 30 to 40 mm, especially 33 to 39 mm. Also the solid core may be of multi-layer structure insofar as it satisfies the above-defined distortion under an applied load of 100 kg.

Next, the inner cover layer **2** is formed mainly of a thermoplastic polyester elastomer.

The thermoplastic polyester elastomer used herein includes polyether ester type multi-block copolymers synthesized from terephthalic acid, 1,4-butane diol, and polytetramethylene glycol (PTMG) or polypropylene glycol (PPG) wherein polybutylene terephthalate (PBT) portions become hard segments and polytetramethylene glycol (PTMG) or polypropylene glycol (PPG) portions become soft segments, for example, Hytrel 4047, G3548W, 4767, and 5577 (by Toray duPont K.K.).

To the thermoplastic polyester elastomer, another polymer such as another elastomer and ionomer resin may be added if necessary. In this regard, the amount of the other polymer added is less than 70 parts by weight, especially less than 50 parts by weight per 100 parts by weight of the thermoplastic polyester elastomer.

Further the inner cover layer **2** composed mainly of the thermoplastic polyester elastomer may contain 0 to about 30% by weight of an inorganic filler such as zinc oxide, barium sulfate, and titanium dioxide.

The inner cover layer should have a Shore D hardness of 28 to 58, especially 30 to 56. A Shore D hardness of less than 28 would detract from restitution whereas hitting feel would be exacerbated above 58.

Further, the inner cover layer **2** should preferably have a specific gravity of 1.05 to 1.4, especially 1.1 to 1.3.

It is noted that the inner cover layer preferably has a gage (**6**) of 0.5 to 3.0 mm, especially 0.9 to 2.5 mm.

On the other hand, the outer cover layer **3** is formed of a thermoplastic polyurethane elastomer.

The thermoplastic polyurethane elastomer used herein has a molecular structure consisting of a high molecular weight polyol compound constituting a soft segment, a monomolecular chain extender constituting a hard segment, and a diisocyanate.

The high molecular weight polyol compound is not critical and may be any of polyester polyols, polyether polyols, copolyester polyols, and polycarbonate polyols. Exemplary polyester polyols include polycaprolactone glycol, poly(ethylene-1,4-adipate) glycol, and poly(butylene-1,4-adipate) glycol; an exemplary copolyester polyol is poly(diethylene glycol adipate) glycol; an exemplary polycarbonate polyol is (hexanediol-1,6-carbonate) glycol; and an exemplary polyether polyol is polyoxetetramethylene glycol. Their number average molecular weight is about 600 to 5,000, preferably 1,000 to 3,000.

As the diisocyanate, aliphatic diisocyanates are preferably used in consideration of the yellowing resistance of the cover. Examples include hexamethylene diisocyanate (HDI), 2,2,4- or 2,4,4-trimethylhexamethylene diisocyanate (TMDI), and lysine diisocyanate (LDI). HDI is especially preferred for its compatibility with another resin upon blending.

The monomolecular chain extender is not critical and may be selected from conventional polyhydric alcohols and amines. Examples include 1,4-butylene glycol, 1,2-ethylene glycol, 1,3-propylene glycol, 1,6-hexamethylene glycol, 1,3-butylene glycol, dicyclohexylmethylmethanediamine (hydrogenated MDA), and isophoronediamine (IPDA).

Of the thermoplastic polyurethane elastomers, those having a tan  $\delta$  peak temperature of lower than  $-15^{\circ}$  C., especially  $-16^{\circ}$  C. to  $-50^{\circ}$  C. as determined by viscoelasticity measurement are preferred in view of softness and resiliency.

As the thermoplastic polyurethane elastomer, there may be used commercially available ones whose diisocyanate component is aliphatic, for example, Pandex T7298 ( $-20^{\circ}$  C.), T7295 ( $-26^{\circ}$  C.), and T7890 ( $-30^{\circ}$  C.) (by Dai-Nihon Ink Chemical Industry K.K.). Note that the numerals in parentheses each represent a tan  $\delta$  peak temperature.

If necessary, another polymer such as another elastomer and ionomer resin may be added to the thermoplastic polyurethane elastomer in an amount of 0 to 60 parts by weight, especially 0 to 50 parts by weight per 100 parts by weight of the thermoplastic polyurethane elastomer.

Further the outer cover layer **3** composed mainly of the thermoplastic polyurethane elastomer may contain less than 30% by weight, especially 1 to 25% by weight of an inorganic filler such as zinc oxide, barium sulfate, and titanium dioxide.

The outer cover layer **3** should have a Shore D hardness of 30 to 55, preferably 32 to 54, more preferably 33 to 53. A Shore D hardness of less than 30 would detract from restitution whereas hitting feel would be exacerbated above 55.

Further, the outer cover layer **3** should preferably have a specific gravity of 1.05 to 1.4, especially 1.07 to 1.35.

The outer cover layer **3** preferably has a gage (**6**) of 0.5 to 2.5 mm, especially 0.9 to 2.4 mm. Durability would become poor below 0.5 mm whereas restitution and hitting feel would become poor above 2.5 mm.

The inner and outer cover layers **2,3** preferably have a total gage (overall cover gage) of 1.0 to 5.5 mm, especially 1.5 to 5.0 mm.

Understandably, the inner and outer cover layers **2,3** may be formed by well-known techniques such as injection molding and compression molding using half shells.

The multi-piece solid golf ball thus obtained should preferably have an inertia moment of at least  $83 \text{ g-cm}^2$ , especially 84 to 90  $\text{g-cm}^2$  as measured by the method described later. An inertia moment of less than  $83 \text{ g-cm}^2$  would lead to the disadvantage that the ball rolling upon putting becomes unsustained and loses straightness.

The outer cover layer **3** is formed with dimples in a conventional manner. With respect to the diameter, weight and other parameters, the golf ball of the invention is constructed in accordance with the Rules of Golf to a diameter of not less than 42.67 mm and a weight of not greater than 45.93 grams.

There has been described a multi-piece solid golf ball featuring an increased flight distance, superior control, pleasant feeling, and improved durability.

## EXAMPLE

Examples of the present invention are given below together with Comparative Examples by way of illustration and not by way of limitation.

### Examples and Comparative Examples

Solid cores of the composition shown in Table 1 were prepared.



TABLE 3-continued

| Outer cover layer (pbw) | Shore D | Specific gravity |     |     |    |      |      |      |      |
|-------------------------|---------|------------------|-----|-----|----|------|------|------|------|
|                         |         |                  | A   | B   | C  | D    | E    | F    | G    |
| Titanium dioxide        | —       | 4.2              | 2.7 | 2.7 | 12 | 5.13 | 5.13 | 5.13 | 5.13 |

PANDEX T7890/T7298: Dai-Nihon Ink Chemical Industry K.K., thermoplastic polyurethane elastomer  
 Himilan: Mitsui duPont Polymers K.K., ionomer resin  
 Surlyn 8120: E. I. duPont, ionomer resin

TABLE 4

|                        |                                     | Example |       |       |       |
|------------------------|-------------------------------------|---------|-------|-------|-------|
|                        |                                     | 1       | 2     | 3     | 4     |
| Core                   | Weight (g)                          | 28.36   | 27.65 | 26.95 | 22.29 |
|                        | Diameter (mm)                       | 36.60   | 36.40 | 36.60 | 34.00 |
|                        | Distortion @100 kg (mm)             | 3.50    | 4.00  | 4.00  | 3.30  |
| Inner cover layer      | Specific gravity                    | 1.105   | 1.095 | 1.050 | 1.083 |
|                        | Type                                | a       | b     | c     | b     |
|                        | Shore D hardness                    | 40      | 47    | 40    | 47    |
|                        | Specific gravity                    | 1.12    | 1.15  | 1.25  | 1.15  |
| Outer cover layer      | Gage (mm)                           | 1.60    | 1.70  | 1.05  | 2.85  |
|                        | Specific gravity                    | 1.18    | 1.18  | 1.26  | 1.18  |
|                        | Gage (mm)                           | 1.45    | 1.45  | 2.00  | 1.50  |
| Ball                   | Shore D hardness                    | 50      | 39    | 39    | 50    |
|                        | Weight (g)                          | 45.3    | 45.3  | 45.3  | 45.3  |
|                        | Diameter (mm)                       | 42.7    | 42.7  | 42.7  | 42.7  |
|                        | Inertia moment (g-cm <sup>2</sup> ) | 84.5    | 84.8  | 86.3  | 85.0  |
| #W1/HS45               | Carry (m)                           | 208.8   | 209.0 | 208.8 | 208.6 |
|                        | Total (m)                           | 222.5   | 223.1 | 222.3 | 222.5 |
|                        | Spin (rpm)                          | 2865    | 2945  | 2918  | 2828  |
|                        | Feeling                             | ○       | ○     | ○     | ○     |
|                        | #SW/HS20 approach spin (rpm)        | 6238    | 6282  | 6256  | 6125  |
| #PT feeling            | ○                                   | ○       | ○     | ○     |       |
| Scraping resistance    | ○                                   | ○       | ○     | ○     |       |
| Consecutive durability | ○                                   | ○       | ○     | ○     |       |

TABLE 5

|                   |                          | Comparative Example |       |       |       |       |       |
|-------------------|--------------------------|---------------------|-------|-------|-------|-------|-------|
|                   |                          | 1                   | 2     | 3     | 4     | 5     | 6     |
| Core              | Weight (g)               | 25.83               | 30.25 | 27.47 | 29.72 | 30.76 | 29.16 |
|                   | Diameter (mm)            | 35.50               | 36.40 | 35.30 | 36.50 | 36.50 | 36.50 |
|                   | Distortion @ 100 kg (mm) | 2.20                | 3.00  | 4.00  | 2.90  | 2.90  | 3.20  |
| Inner cover layer | Specific gravity         | 1.103               | 1.198 | 1.193 | 1.167 | 1.208 | 1.145 |
|                   | Type                     | a                   | d     | a     | a     | e     | f     |
|                   | Shore D hardness         | 40                  | 42    | 40    | 40    | 56    | 62    |
|                   | Specific gravity         | 1.12                | 1.01  | 1.12  | 1.12  | 0.98  | 0.98  |
| Outer cover layer | Gage (mm)                | 1.63                | 1.80  | 1.70  | 1.60  | 1.60  | 1.60  |
|                   | Specific gravity         | 1.18                | 0.98  | 0.98  | 0.98  | 0.98  | 1.18  |
|                   | Gage (mm)                | 1.98                | 1.35  | 2.00  | 1.50  | 1.50  | 1.50  |
| Ball              | Shore D harness          | 50                  | 45    | 62    | 53    | 58    | 50    |
|                   | Weight (g)               | 45.3                | 45.3  | 45.3  | 45.3  | 45.3  | 45.3  |
|                   | Diameter (mm)            | 42.7                | 42.7  | 42.7  | 42.7  | 42.7  | 42.7  |

TABLE 5-continued

| 5                                   | Comparative Example |       |       |       |       |       |
|-------------------------------------|---------------------|-------|-------|-------|-------|-------|
|                                     | 1                   | 2     | 3     | 4     | 5     | 6     |
| Inertia moment (g-cm <sup>2</sup> ) | 84.6                | 81.2  | 81.3  | 82.1  | 80.9  | 83.4  |
| #W1/HS45 Carry (m)                  | 208.1               | 205.3 | 207.9 | 205.8 | 207.9 | 208.1 |
| Total (m)                           | 217.2               | 217.5 | 221.0 | 218.1 | 219.2 | 220.3 |
| Spin (rpm)                          | 3075                | 3001  | 2548  | 2898  | 2689  | 2734  |
| Feeling                             | X                   | ○     | ○     | ○     | ○     | ○     |
| #SW/HS20 approach spin (rpm)        | 6251                | 6236  | 4923  | 6211  | 5632  | 6132  |
| #PT feeling                         | ○                   | ○     | X     | ○     | X     | X     |
| Scraping resistance                 | ○                   | ○     | ○     | ○     | X     |       |
| Consecutive durability              | ○                   | ○     | X     | ○     | ○     | X     |

What is claimed is:

1. A multi-piece solid golf ball comprising: a solid core and a cover consisting of inner and outer layers surrounding the core, said solid core has a distortion of at least 2.8 mm under an applied load of 100 kg, said inner cover layer consisting essentially of a thermoplastic polyester elastomer to a Shore D hardness of 28 to 58, and said outer cover layer consisting essentially of a thermoplastic polyurethane elastomer to a Shore D hardness of 30 to 55.
2. The golf ball of claim 1 wherein the ball as a whole has an inertia moment of at least 83 g-cm<sup>2</sup>.
3. The golf ball of claim 1 wherein up to 30% by weight of an inorganic filler is added to said outer cover layer.
4. The golf ball of any one of claim 1 wherein said inner cover layer contains 0 to 30% by weight of an inorganic filler.
5. The golf ball of any one of claim 1 wherein said outer cover layer has a specific gravity of 1.05 to 1.4.
6. The golf ball of any one of claim 1 wherein said inner cover layer has a specific gravity of 1.05 to 1.4.
7. The golf ball of any one of claim 1 wherein said core has a specific gravity of 0.9 to 1.2.
8. The golf ball of any one of claim 1 wherein said outer cover layer has a gage of 0.5 to 2.5 mm, said inner cover layer has a gage of 0.5 to 3.0 mm, and said cover has a total gage of 1.0 to 5.5 mm.
9. The golf ball of claim 1 wherein said inner cover layer has a Shore D hardness in the range 28 to 56.
10. The golf ball of claim 1 wherein said outer cover layer has a Shore D hardness in the range 33 to 53.
11. The golf ball of claim 1 wherein said outer cover layer consists essentially of a thermoplastic polyurethane elastomer containing less than 30% by weight of an inorganic filler.
12. The golf ball of claim 1 wherein said inner cover layer consists essentially of a thermoplastic polyester elastomer containing less than 30% by weight of an inorganic filler.
13. The golf ball of claim 1, wherein said core has a distortion of a 2.8 to 6.0 under a load of 100 kg.
14. The golf ball of claim 1, wherein said core has a distortion of 2.9 to 5.0 under a load of 100 kg.

\* \* \* \* \*